

## UNITED STATES PATENT OFFICE.

OSCAR F. MULLER, OF MONTCLAIR, NEW JERSEY, ASSIGNOR TO NYANZA COLOR & CHEMICAL CO. INC., OF NEW YORK, N. Y., A CORPORATION OF NEW YORK.

## DELUSTERING OF ARTIFICIAL-SILK FIBERS OR RAYON.

No Drawing.

Application filed July 14, 1928. Serial No. 292,917.

This invention relates to improvements in the treatment of textile fibers and more particularly has for its object the delustering of artificial silk fibers or rayon. It is well known that for many purposes the higher luster of artificial silk or rayon is objectionable and it is, therefore, advisable to improve the appearance of the artificial silk fibers by removing the excessive gloss or delustering same as may be desired. It is important that in such a treatment the strength of the fiber and its adaptability for other uses be not lessened.

By the process hereinafter described I have been enabled to deluster artificial silk fibers to any desired extent without weakening same.

My improved process is as follows:

I treat artificial silk in skein form although piece goods and hosiery may be so treated in a bath of the following composition:

10 parts by weight of commercial green olive oil soap, and 10 parts by weight of medium white glue are dissolved in 100 parts of water. This mixture is heated, 4 parts of paraffin are added, the glue and soap serving as the emulsifying agents for the emulsion of paraffin in water.

Of this paraffin emulsion 1 part is used to 30 40 parts of water and the rayon material is subjected to a bath of this material at a temperature of 90 to 95° F. for a period of about ten minutes. The specific action of the paraffin emulsion on the rayon fibers is to coat the 35 surface of the rayon fiber with a thin layer of adhesive and render same more susceptible to the subsequent treatment with an abrasive. The preliminary treatment of the rayon fiber with this paraffin emulsion is important as it tends to make the fiber much more receptive to the after treatment with an abrasive.

After this treatment the rayon is put into a hydro-extractor to get rid of the superfluous liquid and is washed with water.

Whilst still moist the fiber is then entered 45 into a fresh water bath containing suspended therein infusorial earth or a similar mild abrasive. For this purpose I take from 5 to 10 pounds of infusorial earth for every 100 parts of water and the material is agitated herein at a temperature of from 90 to 95° F. for about thirty minutes or according to the extent of the delustering desired. It should be understood that instead of the paraffin emulsion 55 above mentioned, other emulsions may be

used, and instead of infusorial earth other abrasives such as chalk, kaolin, fuller's earth, talc or zinc oxide may be substituted.

Instead of the paraffin emulsion above mentioned, I have also been enabled to give the fiber 60 an effective preliminary treatment by the use of solutions which will cover the rayon fiber with a satisfactory surface coating so as to make the subsequent treatment with an abrasive effective. As an example of such a solution I will mention a solution of aluminum stearate in carbon tetrachloride.

Having fully described my invention, what I claim is:—

1. A process of delustering artificial silk 70 fibers by treating same with an emulsion of olive oil soap, removing the superfluous liquid and subjecting the material to a bath containing infusorial earth in suspension.

2. A process of delustering artificial silk 75 fibers by treating same with an emulsion of olive oil soap, glue and paraffin, removing the emulsifying liquid and treating the material in a bath containing infusorial earth in suspension.

3. A process of delustering artificial silk 80 fibers by treating same with an emulsion of olive oil soap, glue and paraffin, removing the emulsifying liquid and treating the material in a bath containing a silicious abrasive in suspension.

4. A process of delustering artificial silk 85 fibers by treating same with an emulsion of olive oil soap, glue and paraffin in water, removing the excessive liquid by hydro-extracting 90 and then treating in a suspension of a silicious abrasive in water for a period of thirty minutes at a temperature of approximately 90° F.

5. A process of delustering artificial silk 95 fibers by subjecting same to the action of an emulsion of soap, glue and paraffin in water and then subjecting same to the action of a mineral abrasive suspended in water at approximately 90° F.

6. A process of delustering artificial silk 100 fibers by subjecting same to the action of an emulsion of soap, glue and paraffin in water and then subjecting same to the action of a mineral abrasive suspended in water at approximately 90° F. and for a period of thirty minutes.

7. A process of delustering artificial silk 105 fibers by treating the same with a paraffin emulsion and then subjecting the fiber to a 110

water bath containing an abrasive in suspension.

8. A process of delustering artificial silk fibers by treating the same with a paraffin emulsion and then subjecting the fiber to a water bath containing infusorial earth in suspension.

9. A process of delustering artificial silk fibers by subjecting the fibers to a preliminary coating of a water proofing material and then treating the fibers so coated to the action of an abrasive suspended in water.

10. The process of delustering artificial silk fibers by subjecting the fibers to a preliminary coating of an adhesive material and then subjecting the fibers so coated to the ac-

tion of water having an abrasive in suspension therein.

11. A process of delustering artificial silk fibers by subjecting said fibers to a preliminary coating of an adhesive material and then subjecting said coated fibers to the action of water having infusorial earth in suspension therein.

12. The process of delustering artificial silk fibers by coating the surface of said fibers with an adhesive material and then subjecting said fibers after coating, to a water bath having an abrasive in suspension therein.

In testimony whereof I affix my signature.

OSCAR F. MULLER